



US010995661B2

(12) **United States Patent**  
**Lineton et al.**

(10) **Patent No.:** **US 10,995,661 B2**  
(45) **Date of Patent:** **\*May 4, 2021**

(54) **THERMALLY INSULATED ENGINE  
COMPONENTS USING A CERAMIC  
COATING**

(71) Applicant: **Tenneco Inc.**, Lake Forest, IL (US)

(72) Inventors: **Warran Boyd Lineton**, Chelsea, MI (US); **Miguel Azevedo**, Ann Arbor, MI (US); **Greg Salenbien**, Britton, MI (US)

(73) Assignee: **Tenneco Inc.**, Lake Forest, IL (US)

(\*) Notice: Subject to any disclaimer, the term of this patent is extended or adjusted under 35 U.S.C. 154(b) by 0 days.

This patent is subject to a terminal disclaimer.

(21) Appl. No.: **16/725,533**

(22) Filed: **Dec. 23, 2019**

(65) **Prior Publication Data**

US 2020/0208573 A1 Jul. 2, 2020

**Related U.S. Application Data**

(63) Continuation of application No. 15/354,080, filed on Nov. 17, 2016, now Pat. No. 10,519,854.  
(Continued)

(51) **Int. Cl.**  
**F02B 77/11** (2006.01)  
**C23C 4/126** (2016.01)  
(Continued)

(52) **U.S. Cl.**  
CPC ..... **F02B 77/11** (2013.01); **C23C 4/02** (2013.01); **C23C 4/06** (2013.01); **C23C 4/10** (2013.01);  
(Continued)

(58) **Field of Classification Search**  
CPC ..... F02B 77/11; C23C 4/073; C23C 4/126  
See application file for complete search history.

(56) **References Cited**

U.S. PATENT DOCUMENTS

5,305,726 A \* 4/1994 Scharman ..... C23C 28/345  
123/668  
6,180,262 B1 1/2001 Freling et al.  
(Continued)

FOREIGN PATENT DOCUMENTS

EP 0926254 A2 6/1999  
JP S5484419 U 6/1979  
(Continued)

OTHER PUBLICATIONS

International Search Report, dated Feb. 8, 2017 (PCT/US2016/062649).

(Continued)

*Primary Examiner* — Kevin A Lathers

(74) *Attorney, Agent, or Firm* — Robert L. Stearns;  
Dickinson Wright, PLLC

(57) **ABSTRACT**

A component for exposure to a combustion chamber of a diesel engine and/or exhaust gas, such as a cylinder liner or valve face, is provided. The component includes a thermal barrier coating applied to a body portion formed of steel. A layer of a metal bond material can be applied first, followed by a mixture of the metal bond material and a ceramic material, optionally followed by a layer of the ceramic material. The ceramic material preferably includes at least one of ceria, ceria stabilized zirconia, yttria stabilized zirconia, calcia stabilized zirconia, magnesia stabilized zirconia, and zirconia stabilized by another oxide. The thermal barrier coating is applied by thermal spray or HVOF. The thermal barrier coating has a porosity of 2% by vol. to 25% vol., a thickness of less than 1 mm, and a thermal conductivity of less than 1.00 W/m·K.

**20 Claims, 5 Drawing Sheets**



**Related U.S. Application Data**

(60) Provisional application No. 62/257,993, filed on Nov. 20, 2015.

**(51) Int. Cl.**

*C23C 4/10* (2016.01)  
*C23C 4/18* (2006.01)  
*C23C 4/06* (2016.01)  
*C23C 4/12* (2016.01)  
*C23C 28/00* (2006.01)  
*C23C 4/02* (2006.01)

**(52) U.S. Cl.**

CPC ..... *C23C 4/12* (2013.01); *C23C 4/126* (2016.01); *C23C 4/18* (2013.01); *C23C 28/321* (2013.01); *C23C 28/3215* (2013.01); *C23C 28/3455* (2013.01); *C23C 28/36* (2013.01)

**(56)****References Cited**

## U.S. PATENT DOCUMENTS

6,368,672 B1 4/2002 Thompson et al.  
 10,519,854 B2 \* 12/2019 Lineton ..... C23C 4/02  
 2007/0207328 A1 9/2007 Frost et al.  
 2007/0261663 A1 11/2007 Lineton et al.

## FOREIGN PATENT DOCUMENTS

|    |              |   |         |       |           |
|----|--------------|---|---------|-------|-----------|
| JP | 55019903 A   | * | 2/1980  | ..... | F02F 1/18 |
| JP | H01184261 A  |   | 7/1989  |       |           |
| JP | H08501602 A  |   | 7/1995  |       |           |
| JP | H11124662 A  |   | 5/1999  |       |           |
| JP | 2000273613 A |   | 10/2000 |       |           |

|    |              |         |
|----|--------------|---------|
| JP | 2009536712 A | 10/2009 |
| JP | 2013087721 A | 5/2013  |
| WO | 9408069 A    | 4/1994  |

## OTHER PUBLICATIONS

Oerlikon Metco: Thermal Spray Powder Products: Ceria-Yttria Stabilized Zirconium Oxide HOSP Powder, Aug. 12, 2014, pp. 1-3, retrieved from the Internet Jan. 16, 2017: [https://www.oerlikon.com/ecomaXL/files/oerlikon\\_DSMTS-0038.1\\_CeZrO.pdf&download=1](https://www.oerlikon.com/ecomaXL/files/oerlikon_DSMTS-0038.1_CeZrO.pdf&download=1).

Chunxu Pan et al., Microstructural characteristics in plasma sprayed functionally graded ZrO<sub>2</sub>/NiCrAl coatings, vol. 162, No. 2-3, Jan. 20, 2003, pp. 194-201 (Sections 1-3.1; Tables 1, 2).

International Search Report, dated Feb. 20, 2017 (PCT/US2016/062648).

Jalaludin Helmisyah Ahmad et al, Experimental Study of Ceramic Coated Piston Crown for Compressed Natural Gas Direct Injection Engines, Procedia Engineering, vol. 68, Nov. 18, 2013, pp. 505-511 (Sections 2.1, 3.1; Figure 2; Table 1).

Khor K A et al: "Plasma sprayed functionally graded thermal barrier coatings", Materials Let, Elsevier, Amsterdam, NL, vol. 38, No. 6, Mar. 1, 1999 (Mar. 1, 1999), pp. 437-444, XP004256128, ISSN: 0167-577X, DOI: 10.1016/S0167-577X(98)00203-1, Sections 1-3.2, tables 3-5.

M. B. Beardsley, Final Report of Thick Thermal Barrier Coatings (TTBCs) for Low Emission, High Efficiency Diesel Engine Components, Prepared for Assistant Secretary for Energy Efficiency and Renewable Energy, Office of Transportation Technologies as part of the Ceramic Technology Project of the Materials, Development Program, under contract FC05-97OR22580, Mar. 26, 2006, 144 pages.

Ralph A. Corvino, Ceramic Coating Diesel Engine Combustion Components, 1989, pp. 43-44.

\* cited by examiner

FIG. 1



FIG. 2



FIG. 3



**FIG. 4****EXAMPLE 1:**

50wt% ceramic/25wt% mix/25wt% bond consisting of CSZ/CSZ+bond/bond

| Layer | Component | % by mass |
|-------|-----------|-----------|
| Top   | CSZ       | 50.0      |
|       | YSZ       | 0.0       |
| Mid   | CSZ       | 12.5      |
|       | YSZ       | 0.0       |
|       | Bond      | 12.5      |
| Bond  | Bond only | 25.0      |

**FIG. 5A**

**EXAMPLE 2:**

50wt% ceramic/25wt% mix/25wt% bond consisting of (mix CSZ/YSZ)/(CSZ/YSZ)+bond/bond

| Layer | Component | % by mass |
|-------|-----------|-----------|
| Top   | CSZ       | 25.0      |
|       | YSZ       | 25.0      |
| Mid   | CSZ       | 6.3       |
|       | YSZ       | 6.3       |
|       | Bond      | 12.5      |
| Bond  | Bond only | 25.0      |

**FIG. 5B****EXAMPLE 3:**

50wt% ceramic/25wt% mix/25wt% bond consisting of YSZ/YSZ+bond/bond

| Layer | Component | % by mass |
|-------|-----------|-----------|
| Top   | CSZ       | 0.0       |
|       | YSZ       | 50.0      |
| Mid   | CSZ       | 0.0       |
|       | YSZ       | 12.5      |
|       | Bond      | 12.5      |
| Bond  | Bond only | 25.0      |

**FIG. 5C****EXAMPLE 4:**

Five layer coating transitioning from 100% bond to 100% ceramic

| Layer   | Composition by mass %                |
|---------|--------------------------------------|
| Top CSZ | 20% of total coating, 100;0 CSZ:bond |
| Layer 4 | 20% of total coating, 75;25 CSZ:bond |
| Layer 3 | 20% of total coating, 50;50 CSZ:bond |
| Layer 2 | 20% of total coating, 25;75 CSZ:bond |
| Bond    | 20% of total coating, 0;100 CSZ:bond |

**FIG. 5D**



**FIG. 6**

## 1

**THERMALLY INSULATED ENGINE  
COMPONENTS USING A CERAMIC  
COATING**

**CROSS-REFERENCE TO RELATED  
APPLICATIONS**

This U.S. continuation application claims priority to U.S. utility patent application Ser. No. 15/354,080, filed Nov. 17, 2016, which claims the benefit of U.S. provisional patent application No. 62/257,993, filed Nov. 20, 2015, the entire contents of which are incorporated herein by reference.

**BACKGROUND OF THE INVENTION**

1. Field of the Invention

This invention relates generally to internal combustion engines, including insulated components exposed to combustion chambers and/or exhaust gas of diesel engines, and methods of manufacturing the same.

2. Related Art

Modern heavy duty diesel engines are being pushed towards increased efficiency under emissions and fuel economy legislation. To achieve greater efficiency, the engines must run hotter and at higher peak pressures. Thermal losses through the combustion chamber become problematic under these increased demands. Typically, about 4% to 6% of available fuel energy is lost as heat through the piston into the cooling system. One way to improve engine efficiency is to extract energy from hot combustion gases by turbo-compounding. For example, about 4% to 5% of fuel energy can be extracted from the hot exhaust gases by turbo-compounding.

Another way to improve engine efficiency includes reducing heat losses to the cooling system by insulating components of the engine, for example using insulating layers formed of ceramic materials. One option includes applying a metal bonding layer to a metal surface followed by a ceramic layer. However, the layers are discrete and the ceramic is by its nature porous. Thus, combustion gases can pass through the ceramic and start to oxidize the metal bonding layer at the ceramic/bonding layer interface, causing a weak boundary layer to form and potential failure of the coating over time. In addition, mismatches in thermal expansion coefficients between adjacent layers, and the brittle nature of ceramics, create the risk for delamination and spalling.

Another example is a thermally sprayed coating formed of yttria stabilized zirconia. This material, when used alone, can suffer destabilization through thermal effects and chemical attack in diesel combustion engines. It has also been found that thick ceramic coatings, such as those greater than 500 microns, for example 1 mm, are prone to cracking and failure. Typical aerospace coatings used for jet turbines are oftentimes not suitable because of raw material and deposition costs associated with the highly cyclical nature of the thermal stresses imposed.

**SUMMARY OF THE INVENTION**

One aspect of the invention provides a component for exposure to a combustion chamber of an internal combustion engine, such as a diesel engine, and/or exhaust gas generated by the internal combustion engine. The compo-

## 2

5 nent comprises a body portion formed of metal and a thermal barrier coating applied to the body portion. The thermal barrier coating includes a mixture of a metal material and a ceramic material. The thermal barrier coating has a thickness of less than 1 mm and a thermal conductivity of less than 0.5 W/m·K.

10 According to another embodiment, the component also comprises a body portion formed of metal, and a thermal barrier coating applied to the body portion. The thermal barrier coating includes a mixture of a metal material and a ceramic material. In this embodiment, the thermal barrier coating has a porosity of 2% by vol. to 25% by vol., based on the total volume of the thermal barrier coating. The thermal barrier coating also has a surface roughness Ra of 15 less than 15  $\mu\text{m}$  and a surface roughness Rz of not greater than 110  $\mu\text{m}$ .

20 According to another embodiment, the component also comprises a body portion formed of metal and a thermal barrier coating applied to the body portion. The thermal barrier coating includes a mixture of a metal material and a ceramic material. In this embodiment, the thermal barrier coating has a porosity of 2% by vol. to 25% by vol., based on the total volume of the thermal barrier coating. The thermal barrier coating also has a thermal conductivity of less than 0.5 W/m·K.

**BRIEF DESCRIPTION OF THE DRAWINGS**

30 Other advantages of the present invention will be readily appreciated, as the same becomes better understood by reference to the following detailed description when considered in connection with the accompanying drawings wherein:

35 FIG. 1 is a side cross-sectional view of a combustion chamber of a diesel engine, wherein components exposed to the combustion chamber are coated with a thermal barrier coating according to an example embodiment of the invention;

40 FIG. 2 is an enlarged view of a cylinder liner exposed to the combustion chamber of FIG. 1 with the thermal barrier coating applied to a portion of the cylinder liner;

45 FIG. 3 is an enlarged view of a valve face exposed to the combustion chamber of FIG. 1 with the thermal barrier coating applied to the valve face;

FIG. 4 is an enlarged cross-sectional view showing an example of the thermal barrier coating disposed on the cylinder liner;

50 FIGS. 5A-5D disclose example compositions of the thermal barrier coating; and

FIG. 6 is a cross-sectional view showing an example of the thermal barrier coating disposed on a steel component.

55 **DETAILED DESCRIPTION OF EXAMPLE  
EMBODIMENTS**

One aspect of the invention provides a component of an internal combustion engine 20, such as a heavy duty diesel engine, including a thermal barrier coating 22. The thermal barrier coating 22 prevents heat from passing through the component, and thus can maintain heat in a desired area of the internal combustion engine 20, for example in a fuel-air mixture of a combustion chamber 24 or in exhaust gas, which improves engine efficiency. The thermal barrier coating 22 is also more cost effective and stable, as well as less susceptible to chemical attacks, compared to other coatings used to insulate engine components.

Various different components of the internal combustion engine 20 can be coated with the thermal barrier coating 22. A corresponding U.S. patent application filed on the same day as the present application and claiming priority to the same provisional patent application No. 62/257,993 is directed to application of the thermal barrier coating 22 to a piston 26. However, as shown in FIG. 1, the thermal barrier coating 22 can be applied to one or more other components exposed to the combustion chamber 24, including a cylinder liner 28, cylinder head 30, fuel injector 32, valve seat 34, and valve face 36. Typically, the thermal barrier coating 22 is only applied to a portion of the component exposed to the combustion chamber 24. For example, an entire surface of the component exposed to the combustion chamber 24 could be coated. Alternatively, only a portion of the surface of the component exposed to the combustion chamber 24 is coated. The thermal barrier coating 22 could also be applied to select locations of the surface exposed to the combustion chamber 24, depending on the conditions of the combustion chamber 24 and location of the surface relative to other components.

In the example embodiment of FIG. 1, the thermal barrier coating 22 is only applied to a portion of an inner diameter surface 38 of the cylinder liner 28 located opposite a top land 44 of the piston 26 when the piston 26 is located at top dead center, and the thermal barrier coating 22 is not located at any other location along the inner diameter surface 38, and is not located at any contact surfaces of the cylinder liner 28. FIG. 2 is an enlarged view of the portion of the cylinder liner 28 including the thermal barrier coating 22. In this embodiment, the inner diameter surface 38 includes a groove 40 machined therein. The groove 40 extends along a portion of the length of the cylinder liner 28 from a top edge of the inner diameter surface 38, and the thermal barrier coating 22 is disposed in the groove 40. Also in this example, the length 1 of the groove 40 and the thermal barrier coating 22 is 5 mm to 10 mm wide. In other words, the thermal barrier coating 22 extends 5 mm to 10 mm along the length of the cylinder liner 28. In the example embodiment of FIG. 1, the thermal barrier coating 22 is also applied to the valve face 36. FIG. 3 is an enlarged view of the valve face 36 including the thermal barrier coating 22.

The thermal barrier coating 22 could also be applied to other components of the internal combustion engine 20, or components associated with the internal combustion engine 20, for example other components of a valvetrain, post-combustion chamber, exhaust manifold, and turbocharger. The thermal barrier coating 22 is typically applied to components of a diesel engine directly exposed to hot gasses of the combustion chamber 24 or exhaust gas, and thus high temperatures and pressures, while the engine 20 is running. A body portion 42 of the component is typically formed of steel, such as an AISI 4140 grade or a microalloy 38MnSiVS5, for example, or another metal material. Any steel used to form the body portion 42 does not include phosphate. If any phosphate is present on the surface of the body portion 42, then that phosphate is removed prior to applying the thermal barrier coating 22.

The thermal barrier coating 22 is applied to one or more components of the internal combustion engine 20 or exposed to exhaust gas generated by the internal combustion engine 20, to maintain heat in the combustion chamber 24 or in exhaust gas, and thus increase efficiency of the engine 20. The thermal barrier coating 22 is oftentimes disposed in specific locations, depending on patterns from heat map measurements, in order to modify hot and cold regions of the component. The thermal barrier coating 22 is designed for exposure to the harsh conditions of the combustion chamber

24. For example, the thermal barrier coating 22 can be applied to components of the diesel engine 20 subject to large and oscillating thermal cycles. Such components experience extreme cold start temperatures and can reach up to 700° C. when in contact with combustion gases. There is also temperature cycling from each combustion event of approximately 15 to 20 times a second or more. In addition, pressure swings up to 250 to 300 bar are seen with each combustion cycle.

10 A portion of the thermal barrier coating 22 is formed of a ceramic material 50, specifically at least one oxide, for example ceria, ceria stabilized zirconia, yttria stabilized zirconia, calcia stabilized zirconia, magnesia stabilized zirconia, zirconia stabilized by another oxide, and/or a mixture 15 thereof. The ceramic material 50 has a low thermal conductivity, such as less than 1 W/m·K. When ceria is used in the ceramic material 50, the thermal barrier coating 22 is more stable under the high temperatures, pressures, and other harsh conditions of a diesel engine 20. The composition of 20 the ceramic material 50 including ceria also makes the thermal barrier coating 22 less susceptible to chemical attack than other ceramic coatings, which can suffer destabilization when used alone through thermal effects and chemical attack in diesel combustion engines. Ceria and ceria stabilized 25 zirconia are much more stable under such thermal and chemical conditions. Ceria has a thermal expansion coefficient which is preferably similar to the steel material used to form the body portions 42 of the components to which the thermal barrier coating 22 is applied. The thermal expansion 30 coefficient of ceria at room temperature ranges from 10E-6 to 11E-6, and the thermal expansion coefficient of steel at room temperature ranges from 11E-6 to 14E-6. The similar thermal expansion coefficients help to avoid thermal mismatches that produce stress cracks.

35 Typically, the thermal barrier coating 22 includes the ceramic material 50 in an amount of 70 percent by volume (% by vol.) to 95% by vol., based on the total volume of the thermal barrier coating 22. In one embodiment, the ceramic material 50 used to form the thermal barrier coating 22 includes ceria in an amount of 90 to 100 wt. %, based on the total weight of the ceramic material 50. In another example embodiment, the ceramic material 50 includes ceria stabilized zirconia in an amount of 90 to 100 wt. %, based on the total weight of the ceramic material 50. In another example embodiment, the ceramic material 50 includes yttria stabilized zirconia in an amount of 90 to 100 wt. %, based on the total weight of the ceramic material 50. In yet another example embodiment, the ceramic material 50 includes ceria stabilized zirconia and yttria stabilized zirconia in a total amount of 90 to 100 wt. %, based on the total weight of the ceramic material 50. In another example embodiment, the ceramic material 50 includes magnesia stabilized zirconia, calcia stabilized zirconia, and/or zirconia stabilized by another oxide in an amount of 90 to 100 wt. %, based on the 50 total weight of the ceramic material 50. In other words, any of the oxides can be used alone or in combination in an amount of 90 to 100 wt. %, based on the total weight of the ceramic material 50. In cases where the ceramic material 50 does not consist entirely of the ceria, ceria stabilized zirconia, yttria stabilized zirconia, magnesia stabilized zirconia, calcia stabilized zirconia, and/or zirconia stabilized by another oxide, the remaining portion of the ceramic material 50 typically consists of other oxides and compounds such as aluminum oxide, titanium oxide, chromium oxide, silicon oxide, manganese or cobalt compounds, silicon nitride, and/or functional materials such as pigments or catalysts. For example, according to one embodiment, a catalyst is 55 60 65

added to the thermal barrier coating 22 to modify combustion. A color compound can also be added to the thermal barrier coating 22. According to one example embodiment, thermal barrier coating 22 is a tan color, but could be other colors, such as blue or red.

According to one embodiment, wherein the ceramic material 50 includes ceria stabilized zirconia, the ceramic material 50 includes the ceria in an amount of 20 wt. % to 25 wt. % and the zirconia in an amount of 75 wt. % to 80 wt. %, based on the total amount of ceria stabilized zirconia in the ceramic material 50. Alternatively, the ceramic material 50 can include up to 3 wt. % yttria, and the amount of zirconia is reduced accordingly. In this embodiment, the ceria stabilized zirconia is provided in the form of particles having a nominal particle size of 11  $\mu\text{m}$  to 125  $\mu\text{m}$ . Preferably, 90 wt. % of the ceria stabilized zirconia particles have a nominal particle size less than 90  $\mu\text{m}$ , 50 wt. % of the ceria stabilized zirconia particles have a nominal particle size less than 50  $\mu\text{m}$ , and 10 wt. % of the ceria stabilized zirconia particles have a nominal particle size less than 25  $\mu\text{m}$ .

According to another example embodiment, wherein the ceramic material 50 includes yttria stabilized zirconia, the ceramic material 50 includes the yttria in an amount of 7 wt. % to 9 wt. %, and the zirconia in an amount of 91 wt. % to 93 wt. %, based on the amount of yttria stabilized zirconia in the ceramic material 50. In this embodiment, the yttria stabilized zirconia is provided in the form of particles having a nominal particle size of 11  $\mu\text{m}$  to 125  $\mu\text{m}$ . Preferably, 90 wt. % of the yttria stabilized zirconia particles have a nominal particle size less than 90  $\mu\text{m}$ , 50 wt. % of the yttria stabilized zirconia particles have a nominal particle size less than 50  $\mu\text{m}$ , and 10 wt. % of the yttria stabilized zirconia particles have a nominal particle size less than 25  $\mu\text{m}$ .

According to another example embodiment, wherein the ceramic material 50 includes a mixture of ceria stabilized zirconia and yttria stabilized zirconia, the ceramic material 50 includes the ceria stabilized zirconia in an amount of 5 wt. % to 95 wt. %, and the yttria stabilized zirconia in an amount of 5 wt. % to 95 wt. %, based on the total amount of the mixture present in the ceramic material 50. In this embodiment, the ceria stabilized zirconia is provided in the form of particles having a nominal particle size of 11  $\mu\text{m}$  to 125  $\mu\text{m}$ . Preferably, 90 wt. % of the ceria stabilized zirconia particles have a particle size less than 90  $\mu\text{m}$ , 50 wt. % of the ceria stabilized zirconia particles have a particle size less than 50  $\mu\text{m}$ , and 10 wt. % of the ceria stabilized zirconia particles have a particle size less than 25  $\mu\text{m}$ . The yttria stabilized zirconia is also provided in the form of particles having a nominal particle size of 11  $\mu\text{m}$  to 125  $\mu\text{m}$ . Preferably, 90 wt. % of the yttria stabilized zirconia particles have a particle size less than 109  $\mu\text{m}$ , 50 wt. % of the yttria stabilized zirconia particles have a particle size less than 28  $\mu\text{m}$ . When the ceramic material 50 includes the mixture of ceria stabilized zirconia and yttria stabilized zirconia, the ceramic material can be formed by adding 5 wt. % to 95 wt. % of ceria stabilized zirconia to the balance of yttria stabilized zirconia in the total 100 wt. % mixture.

According to yet another example embodiment, wherein the ceramic material 50 includes calcia stabilized zirconia, the ceramic material 50 includes the calcia in an amount of 4.5 wt. % to 5.5 wt. %, and the zirconia in an amount of 91.5 wt. %, with the balance consisting of other oxides in the ceramic material 50. In this embodiment, the calcia stabilized zirconia is provided in the form of particles having a nominal particle size range of 11  $\mu\text{m}$  to 90  $\mu\text{m}$ . Preferably,

the calcia stabilized zirconia particles contain a maximum of 7 wt. % with particle size greater than 45  $\mu\text{m}$  and up to 65 wt. % of particles less than 45  $\mu\text{m}$ .

According to yet another example embodiment, wherein the ceramic material 50 includes magnesia stabilized zirconia, the ceramic material 50 includes the magnesia in an amount of 15 wt. % to 30 wt. %, with the balance consisting of zirconia. In this embodiment, the magnesia stabilized zirconia is provided in the form of particles having a nominal particle size of 11  $\mu\text{m}$  to 90  $\mu\text{m}$ . Preferably, 15 wt. % of the magnesia stabilized zirconia particles have a particle size less than 88  $\mu\text{m}$ .

Other oxides or mixtures of oxides may be used to stabilize the ceramic material 50. The amount of other oxide or mixed oxides is typically in the range 5 wt. % to 38 wt. % and the nominal particle size range of the stabilized ceramic material 50 is 1  $\mu\text{m}$  to 125  $\mu\text{m}$ .

The porosity of the ceramic material 50 is typically controlled to reduce the thermal conductivity of the thermal barrier coating 22. When a thermal spray method is used to apply the thermal barrier coating 22, the porosity of the ceramic material 50 is typically less than 25% by vol., such as 2% by vol. to 25% by vol., preferably 5% by vol. to 15% by vol., and more preferably 8% by vol. to 10% by vol., based on the total volume of the ceramic material 50. However, if a vacuum method is used to apply the thermal barrier coating 22, then the porosity is typically less than 5% by vol., based on the total volume of the ceramic material 50. The porosity of the entire thermal barrier coating 22 can also be 2% by vol. to 25% by vol., but is typically greater than 5% by vol. to 25% by vol., preferably 5% by vol. to 15% by vol., and most preferably 8% by vol. to 10% by vol., based on the total volume of the thermal barrier coating 22. The pores of the thermal barrier coating 22 are typically concentrated in the ceramic regions. The porosity of the thermal barrier coating 22 contributes to the reduced thermal conductivity of the thermal barrier coating 22.

The thermal barrier coating 22 is also applied in a gradient structure 51 to avoid discrete metal/ceramic interfaces. In other words, the gradient structure 51 avoids sharp interfaces. Thus, the thermal barrier coating 22 is less likely to de-bond during service. The gradient structure 51 of the thermal barrier coating 22 is formed by first applying a metal bond material 52 to the component, followed by a mixture of the metal bond material 52 and ceramic material 50, and then the ceramic material 50.

The composition of the metal bond material 52 can be the same as the powder used to form the body portion 42 of the component, for example a steel powder. Alternatively the metal bond material 52 can comprise a high performance superalloy, such as those used in coatings of jet turbines. According to example embodiments, the metal bond material 52 includes or consists of at least one of alloy selected from the group consisting of CoNiCrAlY, NiCrAlY, NiCr, NiAl, NiCrAl, NiAlMo, and NiTi. The thermal barrier coating 22 typically includes the metal bond material 52 in an amount of 5% by vol. to 33% by vol. %, more preferably 10% by vol. to 33% by vol., most preferably 20% by vol. to 33% by vol., based on the total volume of the thermal barrier coating 22. The metal bond material 52 is provided in the form of particles having a particle size of -140 mesh (<105  $\mu\text{m}$ ), preferably -170 mesh 90  $\mu\text{m}$ ), more preferably -200 mesh 74  $\mu\text{m}$ ), and most preferably -400 mesh (<37  $\mu\text{m}$ ). According to one example embodiment, the thickness of the metal bond material 52 ranges from 30 microns to 1 mm. The thickness limit of the metal bond material 52 is dictated by the particle size of the metal bond material 52. A low

thickness is oftentimes preferred to reduce the risk of delamination of the thermal barrier coating 22.

The gradient structure 51 is formed by gradually transitioning from 100% metal bond material 52 to 100% ceramic material 50. The thermal barrier coating 22 includes the metal bond material 52 applied to the body portion 26, followed by increasing amounts of the ceramic material 50 and reduced amounts of the metal bond material 52. The transition function of the gradient structure 51 can be linear, exponential, parabolic, Gaussian, binomial, or could follow another equation relating composition average to position.

The uppermost portion of the thermal barrier coating 22 is formed entirely of the ceramic material 50. The gradient structure 51 helps to mitigate stress build up through thermal mismatches and reduces the tendency to form a continuous weak oxide boundary layer at the interface of the ceramic material 50 and the metal bond material 52.

According to one embodiment, as shown in FIG. 4, the lowermost portion of the thermal barrier coating 22 applied directly to the surface of the body portion 42, such as the inner diameter surface 38 of the cylinder liner 28, consists of the metal bond material 52. Typically, 5% to 20% of the entire thickness of the thermal barrier coating 22 is formed of 100% metal bond material 52. In addition, the uppermost portion of the thermal barrier coating 22 can consist of the ceramic material 50. For example, 5% to 50% of the entire thickness of the thermal barrier coating 22 could be formed of 100% ceramic material 50. The gradient structure 51 of the thermal barrier coating 22 which continuously transitions from the 100% metal bond material 52 to the 100% ceramic material 50 is located therebetween. Typically, 30% to 90% of the entire thickness of the thermal barrier coating 22 is formed of, or consists of, the gradient structure 51. It is also possible that 10% to 90% of the entire thickness of the thermal barrier coating 22 is formed of a layer of the metal bond layer 52, up to 80% of the thickness of the thermal barrier coating 22 is formed of the gradient structure 51, and 10% to 90% of the entire thickness of the thermal barrier coating 22 is formed of a layer of the ceramic material 50. FIG. 4 is an enlarged cross-sectional view showing an example of the thermal barrier coating 22 disposed on the inner diameter surface 38 of the cylinder liner 28. Example compositions of the thermal barrier coating 22 including ceria stabilized zirconia (CSZ), yttria stabilized zirconia (YSZ), and metal bond material (Bond) are disclosed in FIGS. 5A-5D. FIG. 6 is a cross-sectional view showing an example of the thermal barrier coating 22 disposed on the steel body portion 42.

In its as-sprayed form, the thermal barrier coating 22 typically has a surface roughness Ra of less than 15  $\mu\text{m}$ , and a surface roughness Rz of not greater than <110  $\mu\text{m}$ . The thermal barrier coating 22 can be smoothed. At least one additional metal layer, at least one additional layer of the metal bonding material 52, or at least one other layer, could be applied to the outermost surface of the thermal barrier coating 22. When the additional layer or layers are applied, the outermost surface formed by the additional material could also have the surface roughness Ra of less than 15  $\mu\text{m}$ , and a surface roughness Rz of not greater than <110  $\mu\text{m}$ . Roughness can affect combustion by trapping fuel in cavities on the surface of the coating. It is desirable to avoid coated surfaces rougher than the examples described herein.

The thermal barrier coating 22 has a low thermal conductivity to reduce heat flow through the thermal barrier coating 22. Typically, the thermal conductivity of the thermal barrier coating 22 having a thickness of less than 1 mm, is less than 1.00 W/m·K, preferably less than 0.5 W/m·K,

and most preferably not greater than 0.23 W/m·K. The specific heat capacity of the thermal barrier coating 22 depends on the specific composition used, but typically ranges from 480 J/kg·K to 610 J/kg·K at temperatures between 40 and 700°C. The low thermal conductivity of the thermal barrier coating 22 is achieved by the relatively high porosity of the ceramic material 50. Due to the composition and low thermal conductivity of the thermal barrier coating 22, the thickness of the thermal barrier coating 22 can be reduced, which reduces the risk of cracks or spalling, while achieving the same level of insulation relative to comparative coatings of greater thickness. It is noted that the advantageous low thermal conductivity of the thermal barrier coating 22 is not expected. When the ceramic material 50 of the thermal barrier coating 22 includes ceria stabilized zirconia, the thermal conductivity is especially low.

The bond strength of the thermal barrier coating 22 is also increased due to the gradient structure 51 present in the thermal barrier coating 22 and the composition of the metal used to form the component. The bond strength of the thermal barrier coating 22 having a thickness of 0.38 mm is typically at least 2000 psi when tested according to ASTM C633.

The thermal barrier coating 22 with the gradient structure 51 can be compared to a comparative coating having a two layer structure, which is typically less successful than the thermal barrier coating 22 with the gradient structure 51. The comparative coating includes a metal bond layer applied to a metal substrate followed by a ceramic layer with discrete interfaces through the coating. In this case, combustion gases can pass through the porous ceramic layer and can begin to oxidize the bond layer at the ceramic/bond layer interface. The oxidation causes a weak boundary layer to form, which harms the performance of the coating.

However, the thermal barrier coating 22 with the gradient structure 51 can provide numerous advantages. The thermal barrier coating 22 is applied to at least a portion of the surface of the component exposed to the combustion chamber 24 or the exhaust gas generated by the internal combustion engine 20 to provide a reduction in heat flow through the component. The reduction in heat flow is typically at least 50%, relative to the same component without the thermal barrier coating 22. By reducing heat flow through the component, more heat is retained in the fuel-air mixture of the combustion chamber and/or exhaust gas produced by the engine, which leads to improved engine efficiency and performance.

The thermal barrier coating 22 of the present invention has been found to adhere well to the steel body portion 42. However, for additional mechanical anchoring, the surfaces of the body portion 42 to which the thermal barrier coating 22 is applied is typically free of any edge or feature having a radius of less than 0.1 mm. In other words, the surfaces of the component to which the thermal barrier coating 22 is preferably free of any sharp edges or corners. According to one example embodiment, the body portion 42 includes a broken edge or chamfer machined along its surface. The chamfer allows the thermal barrier coating 22 to radially lock to the body portion 42. Alternatively, at least one pocket, recess, or round edge could be machined along the surface of the body portion 42. These features help to avoid stress concentrations in the thermal sprayed coating 22 and avoid sharp corners or edges that could cause coating failure. The machined pockets or recesses also mechanically lock the coating 22 in place, again reducing the probability of delamination failure.

Another aspect of the invention provides a method of manufacturing the coated component for use in the internal combustion engine 20, for example a diesel engine. The component, which is typically formed of steel, can be manufactured according to various different methods, such as forging, casting, and/or welding. As discussed above, the thermal barrier coating 22 can be applied to various different components exposed to the combustion chamber 24 or the exhaust gas generated by the internal combustion engine 20, and those components can comprise various different designs. Prior to applying the thermal barrier coating 22 to the body portion 42, any phosphate or other material located on the surface to which the thermal barrier coating 22 is applied must be removed.

The method next includes applying the thermal barrier coating 22 to the body portion 42 of the component. The thermal barrier coating 22 can be applied to the entire surface of the component exposed to the combustion chamber or the exhaust gases, or only a portion of that surface. The ceramic material 50 and metal bond material 52 are provided in the form of particles or powders. The particles can be hollow spheres, spray dried, spray dried and sintered, sol-gel, fused, and/or crushed. For example, as shown in FIGS. 1-3, the thermal barrier coating 22 is applied to the portion of the cylinder liner 28 and the valve face 36.

In the example embodiment, the method includes applying the metal bond material 52 and the ceramic material 50 by a thermal or kinetic method. According to one embodiment, a thermal spray technique, such as plasma spraying, flame spraying, or wire arc spraying, is used to form the thermal barrier coating 22. High velocity oxy-fuel (HVOF) spraying is a preferred example of a kinetic method that gives a denser coating. Other methods of applying the thermal barrier coating 22 to the component can also be used. For example, the thermal barrier coating 22 could be applied by a vacuum method, such as physical vapor deposition or chemical vapor deposition. According to one embodiment, HVOF is used to apply a dense layer of the metal bond material 52 to the component, and a thermal spray technique, such as plasma spray, is used to apply the gradient structure 51 and the layer of ceramic material 50. Also, the gradient structure 51 can be applied by changing feed rates of twin powder feeders while the plasma sprayed coating is being applied.

The example method begins by spraying the metal bond material 52 in an amount of 100 wt. % and the ceramic material 50 in an amount of 0 wt. %, based on the total weight of the materials being sprayed. Throughout the spraying process, an increasing amount of ceramic material 50 is added to the composition, while the amount of metal bond material 52 is reduced. Thus, as shown in FIG. 4, the composition of the thermal barrier coating 22 gradually changes from 100% metal bond material 52 along the component to 100% ceramic material 50 at a top surface 58 of the thermal barrier coating 22. Multiple powder feeders are typically used to apply the thermal barrier coating 22, and their feed rates are adjusted to achieve the gradient structure 51. The gradient structure 51 of the thermal barrier coating 22 is achieved during the thermal spray process.

The thermal barrier coating 22 can be applied to the entire component, or a portion thereof, for example only the surface exposed to the combustion chamber 24 or exhaust gas, or only a portion of that surface. Non-coated regions of the component can be masked during the step of applying the thermal barrier coating 22. The mask can be a re-usable and removal material applied adjacent the region being coated. Masking can also be used to introduce graphics in

the thermal barrier coating 22. In addition, after the thermal barrier coating 22 is applied, the coating edges are blended, and sharp corners or edges are reduced to avoid high stress regions.

As shown in FIG. 4, the thermal barrier coating 22 has a thickness  $t$  extending from the surface of the body portion 42 of the component, for example the inner diameter surface 38 of the cylinder liner 28, to the top surface 58. According to example embodiments, the thermal barrier coating 22 is applied to a total thickness  $t$  of not greater than 1.0 mm, or not greater than 0.7 mm, preferably not greater than 0.5 mm, and most preferably not greater than 0.380 mm. In the example embodiment of FIGS. 1 and 2, the total thickness  $t$  of the thermal barrier coating 22 disposed along the inner diameter surface 38 of the cylinder liner 28 is 0.380 mm. This total thickness  $t$  preferably includes the total thickness of the thermal barrier coating 22 and also any additional or sealant layer applied to the uppermost surface of the thermal barrier coating 22. However, the total thickness  $t$  could be greater when the additional layers are used.

The thickness  $t$  can be uniform along the entire surface of the component, but typically the thickness  $t$  varies along the surface of the component, especially if the surface has a complex shape. In certain regions of the component, for example where the component is subject to less heat and pressure, the thickness  $t$  of the thermal barrier coating 22 can be as low as 0.020 mm to 0.030 mm. In other regions of the component, for example regions which are subjected to the highest temperatures and pressures, the thickness  $t$  of the thermal barrier coating 22 is increased. For example, the method can include aligning the component 20 in a specific location relative to the spray gun and fixture, fixing the component to prevent rotation, using a scanning spray gun in a line, and varying the speed of the spray or other technique used to apply the thermal barrier coating 22 to adjust the thickness  $t$  of the thermal barrier coating 22 over different regions of the component.

In addition, more than one layer of the thermal barrier coating 22, such as 5-10 layers, having the same or different compositions, could be applied to the component. Furthermore, coatings having other compositions could be applied to the component in addition to the thermal barrier coating 22. According to one example embodiment, an additional metal layer, such as an electroless nickel layer, is applied over the thermal barrier coating 22 to provide a seal against fuel absorption, prevent thermally grown oxides, and prevent chemical degradation of the ceramic material 50. The thickness of the additional metal layer is preferably from 1 to 50 microns. If the additional metal layer is present, the porosity of the thermal barrier coating 22 could be increased. Alternatively, an additional layer of the metal bonding material 52 can be applied over the ceramic material 50 of the thermal barrier coating 22.

Prior to applying the thermal barrier coating 22, the surface of the component to which the thermal barrier coating 22 is applied is washed in solvent to remove contamination. Next, the method typically includes removing any edge or feature having a radius of less than 0.1 mm. The method can also include forming the broken edges or chamfer 56, or another feature that aids in mechanical locking of the thermal barrier coating 22 to the component and reduce stress risers, in the component. These features can be formed by machining, for example by turning, milling or any other appropriate means. The method can also include grit blasting surfaces of the component prior to applying the thermal barrier coating 22 to improve adhesion of the thermal barrier coating 22.

## 11

After the thermal barrier coating 22 is applied to the component, the coated component can be abraded to remove asperities and achieve a smooth surface. In the example embodiment of FIGS. 1 and 2, the thermal barrier coating 22 applied to the cylinder liner 28 requires post-finishing, for example by machining or honing. The method can also include forming a marking on the surface of the thermal barrier coating 22 for the purposes of identification of the coated component when the component is used in the market. The step of forming the marking typically involves re-melting the thermal barrier coating 22 with a laser. According to other embodiments, an additional layer of graphite, thermal paint, or polymer is applied over the thermal barrier coating 22. If the polymer coating is used, the polymer burns off during use of the component in the engine 20. The method can include additional assembly steps, such as washing and drying, adding rust preventative and also packaging. Any post-treatment of the coated component must be compatible with the thermal barrier coating 22.

Obviously, many modifications and variations of the present invention are possible in light of the above teachings and may be practiced otherwise than as specifically described while within the scope of the following claims.

The invention claimed is:

1. A component for exposure to a combustion chamber of an internal combustion engine and/or exhaust gas generated by the internal combustion engine, comprising:

a body portion formed of metal;

a thermal barrier coating applied to said body portion; said thermal barrier coating including a metal material and a ceramic material;

said ceramic material including ceria stabilized zirconia; and

said thermal barrier coating having a thickness of less than less than 1 mm.

2. The component of claim 1, wherein said thermal barrier coating has a porosity of 2% by vol. to 25% by vol., based on the total volume of said thermal barrier coating.

3. The component of claim 1, wherein said ceramic material of said thermal barrier coating further includes at least one of yttria stabilized zirconia, calcia stabilized zirconia, and magnesia stabilized zirconia.

4. The component of claim 1, wherein said ceramic material consists of ceria stabilized zirconia.

5. The component of claim 1, wherein said metal material is applied directly to said body portion formed of metal, and 5% to 20% of said thickness of said thermal barrier coating consists of said metal material applied directly to said body portion;

said thermal barrier coating includes a gradient structure applied directly to said metal material, said gradient structure includes metal and said ceramic material, the amount of said ceramic material present in said gradient structure increases continuously toward a top surface of said thermal barrier coating; and

said thermal barrier coating includes a top layer of said ceramic material applied directly to said gradient structure and extending to said top surface, and 5% to 50% of said thickness of said thermal barrier coating consists of said top layer of said ceramic material.

6. The component of claim 1, wherein said metal material includes at least one alloy selected from the group consisting of CoNiCrAlY, NiCrAlY, NiCr, NiAl, NiCrAl, NiAlMo, and NiTi.

## 12

7. The component of claim 1, wherein a surface of said body portion to which said thermal barrier coating is applied is free of any feature having a radius of less than 0.1 mm.

8. The component of claim 1, wherein said thermal barrier coating applied to a surface of said body portion has a bond strength of at least 2000 psi when tested according to ASTM C633.

9. The component of claim 1, wherein said thermal barrier coating is applied to a surface of said body portion exposed to said combustion chamber and/or said exhaust gas, and said thermal barrier coating is applied a first portion of said surface and not applied to a second portion of said surface.

10. The component of claim 1, wherein said component is selected from the group consisting of a cylinder liner, a cylinder head, a fuel injector, a valve seat, and a valve face.

11. The component of claim 10, wherein said component is said cylinder liner, said cylinder liner includes an inner diameter surface, and said thermal barrier coating is applied to a first portion of said inner diameter surface located opposite a top land of a piston when the piston is located at top dead center and not applied to a second portion of said inner diameter surface located below said first portion.

12. The component of claim 11, wherein said inner diameter surface of said cylinder liner includes a groove, and said thermal barrier coating is disposed in said groove.

13. The component of claim 1, wherein said component is selected from the group consisting of a valvetrain, a surface of a post-combustion chamber, an exhaust manifold, and a turbocharger.

14. The component of claim 1, wherein at least one additional layer formed of metal is applied to said thermal barrier coating.

15. The component of claim 14, wherein said metal of said at least one additional layer is the same as said metal material of said thermal barrier coating.

16. The component of claim 1, wherein said thermal barrier coating has a surface roughness Ra of less than 15  $\mu\text{m}$  and a surface roughness Rz of not greater than 110  $\mu\text{m}$ .

17. A component for exposure to a combustion chamber of an internal combustion engine and/or exhaust gas generated by the internal combustion engine, comprising:

a body portion formed of metal;

a thermal barrier coating applied to said body portion; said thermal barrier coating including ceria stabilized zirconia; and

said thermal barrier coating having a surface roughness Ra of less than 15  $\mu\text{m}$  and a surface roughness Rz of not greater than 110  $\mu\text{m}$ .

18. The component of claim 17, wherein said component is selected from the group consisting of a valvetrain, a surface of a post-combustion chamber, an exhaust manifold, and a turbocharger.

19. A component for exposure to a combustion chamber of an internal combustion engine and/or exhaust gas generated by the internal combustion engine, comprising:

a body portion formed of metal;

a thermal barrier coating applied to said body portion; said thermal barrier coating including ceria stabilized zirconia;

said thermal barrier coating having a porosity of 2% by vol. to 25% by vol., based on the total volume of said thermal barrier coating.

20. The component of claim 19, wherein said component is selected from the group consisting of a valvetrain, a surface of a post-combustion chamber, an exhaust manifold, and a turbocharger.